

June 20, 1944.

E. N. SANDERS

2,351,710

COLD-DRAWING PIPE AND TUBE

Filed March 5, 1941

FIG. 1.



FIG. 2.



Inventor:

ELMER N. SANDERS,  
by: *John E. Jackson*  
his Attorney.

## UNITED STATES PATENT OFFICE

2,351,710

## COLD-DRAWING PIPES AND TUBES

Elmer N. Sanders, Mount Lebanon, Pa., assignor  
to National Tube Company, a corporation of  
New Jersey

Application March 5, 1941, Serial No. 381,902

2 Claims. (Cl. 205—8)

This invention relates to the manufacture of attenuated metallic articles such as pipes and tubes, and more particularly to the cold-drawing thereof.

Heretofore the common manner of lubricating tubing for cold-drawing has been to apply thereto a water-bearing mixture of flour and tallow by dipping bundles of the tubing in tanks containing such compound. After this, the tubing was either placed on drying racks for sufficient time for most of the water to evaporate, or the moisture was driven therefrom by running the tubing through a continuous drying oven. As is readily apparent, the first-mentioned drying method was very slow and the second quite expensive. In addition, the water in the compound caused an oxide to form on the pipe, necessitating pickling, and frequently resulted in localized corrosion or etch-pitting which seriously affected the quality and appearance of the tubing and caused excessive rejections.

The present invention comprises a method of cold-drawing which is calculated to overcome the foregoing difficulties in present-day methods, which include slow and expensive lubricant drying periods, rusting or corrosion causing extra pickling operations, and etch-pitting causing poor surface and many rejections.

According to the teachings of the present invention, the hot-rolled tubing is pickled (placed in an acid bath to remove the scale) and after passing through a neutralizing and washing bath is taken directly to the draw-bench. Here the pickled and washed tubing is drawn through a die and over an interiorly disposed mandrel to reduce the outer diameter and/or wall thickness. An oil base non-water-bearing lubricant is directed onto the exterior and interior of the tubing adjacent to the inlet side of the die. The oil base non-water-bearing lubricant gives the tubing a rust preventative coating which prevents rusting should there be any appreciable delay before the tubing can be annealed.

After the drawing operation, the tubing is conventionally annealed (low temperature heat treatment which removes drawing strains and hardness). This is preferably done in an inert or reducing atmosphere to prevent scaling, and accordingly no pickling is necessary in this method except the initial pickling prior to the first drawing. Ordinarily the hot-rolled tube must be drawn several times to attain the desired diameter and wall thickness, and according to the present method the annealed tube can be immediately redrawn in the foregoing manner and

annealed in sequence without intermediate pickling or other treatment until the desired dimensions are obtained. By materially reducing the time cycle for one drawing until the next drawing, there is obtained a great saving in the cost of the finished tube.

Referring to the accompanying drawing, there is illustrated therein a preferred form of apparatus which may be employed for practicing the method described hereinbefore.

More specifically:

Figure 1 is a side elevation of a part of the apparatus of the present invention;

Figure 2 is an enlarged fragmentary elevation, mostly in section, and illustrating those elements of the apparatus which are disposed interiorly of the tubular workpiece.

Referring more particularly to the drawing, the numeral 1 generally designates a draw-bench of a type widely used in the cold-drawing of metallic pipes and tubes and adjacent one end of which there is disposed the usual drawing die 2.

According to the teachings of the present invention there is provided adjacent the drawing die 2, and on the entry side thereof, a spray ring 3 which receives lubricant under pressure in a manner which will be more fully described hereinafter and ejects the same around the periphery of the workpiece.

Disposed within the pipe or tube to be cold-drawn, which is designated hereinafter at X, is a hollow mandrel bar 4 carrying on its forward end a mandrel 5 having an enlarged cylindrical head 7 for disposal immediately opposite the working surfaces of the drawing die 2. As shown at 8 in Figure 2, the forward end of the enlarged cylindrical head 7 of the mandrel is relieved or beveled.

The extreme forward end of the hollow mandrel bar 4 and the extreme rearward end of the mandrel 5 are of substantially the same diameter and are center bored and screw threaded as shown at 11 to accommodate between them a threaded stud 12 whereby the mandrel is rigidly secured to the hollow mandrel bar, thus permitting easy replacement of the mandrel with its enlarged cylindrical head 7 when such is desired.

The rearward end of the hollow mandrel bar 4 carries an integral collar 14 which by means of nuts 16 and 17 is secured to the forward end of a draw-bench anchor 19. This anchor 19 carries a fitting 21 which is connected to a supply of lubricant under pressure by means of a flexible tube 23. This fitting 21 is provided with

passage 25 which communicates with radial passages 26 in the forward end of the draw-bench anchor 19, the said radial passages 26 communicating in turn with a central bore 27 which extends to the exterior of the forward end of the said draw-bench anchor and communicates with the rearward end of the bore of the hollow mandrel bar 4.

At the forward end of the hollow mandrel bar 4 and to the rear of the threaded stud 12 is a series of apertures 28 which communicate with the central bore 27 and extend forwardly and convergently with respect to the mandrel 5 for the purpose of supplying lubricant to the exterior of the latter.

Due to the foregoing construction and arrangement, the hollow mandrel bar 4 may be quickly replaced when necessary without disturbing the piping connection afforded by the fitting 21 and flexible tube 23.

Referring more particularly to Figure 1, beneath the draw-bench 1 and the drawing die 2 there is disposed a sump 30 for the reception of lubricant stripped from the tube by the drawing die 2 and the hollow mandrel bar 4. This sump 30 has disposed thereabove a pair of sloping trough plates 31 and 32 which extend in both directions along the draw bench 1, as shown at 33 and 34 respectively, to provide receiving surfaces for the lubricant; thus the lubricant is collected from both the front and back of the drawing die 2. A pressure pump 36 is connected with the sump 30 by means of a suction line 37 and has connected therewith a piping system 38 which delivers lubricant to the flexible hose 23 referred to hereinbefore and also the spray ring 3 which is disposed around the aperture of the drawing die 2. Disposed in the piping system 38 is a pressure relief valve 41 which permits excess lubricant to return to the sump 30, whereby there is maintained a uniform pressure in the lubricating system. Control valves are provided as indicated at 44 and 45, to permit the separate regulation of supply of lubricant to both the flexible hose 23 and the cylindrical ring 5.

The operation of drawing a tube is as follows:

The valves 44 and 45 are closed or throttled down to permit only a small flow of lubricant. The hollow mandrel bar 4 is pushed back axially about two feet to clear the drawing die 2, and the end of the mandrel 5 is moved either vertically or horizontally away from the pass line and a tube is threaded over the mandrel and mandrel bar until the pointed or reduced end reaches the mandrel. Enough lubricant is admitted to the mandrel to assure its having flooded the inside

5 of the tube past the mandrel, which is always somewhat smaller than the inside of the un-drawn tube. The tube and mandrel are then pushed back into the pass line and moved axially until the point extends through the die. The valves 44 and 45 are then opened and lubricant floods both the outside and inside surfaces of the tube near the die and mandrel. A plier 50 grips the pointed end of the tube extending through the die and the tube is drawn through the die and over the mandrel.

It will be noted that as the tube is drawn down tight on the mandrel 5, no excess lubricant will pass the mandrel or through the die, during the 10 drawing operation. Just before the tube is completely drawn, the valves 44 and 45 are closed, thus stopping or reducing the flow of lubricant until the next tube is ready for its passage through the die.

15 While I have shown and described certain specific embodiments of my invention, I do not intend to be specifically limited thereto, since many departures may be made from the embodiments disclosed herein without departing from the spirit 20 of the invention or the scope of the appended claims.

I claim:

1. The method of producing cold-drawn tubing, which comprises providing a hot-rolled pickled tube which has been subjected to a neutralizing washing operation, then immediately after the washing operation transferring the tube directly to a draw-bench and there passing it through a die and over a mandrel disposed interiorly of said die and tube, applying a liquid non-water-bearing lubricant simultaneously to both the interior and the exterior surfaces of 30 said tube as it is being drawn through said die and prior to their passage therethrough.

35 2. The method of producing cold-drawn tubing, which comprises providing a hot-rolled pickled tube which has been subjected to a neutralizing washing operation, then immediately after the washing operation transferring the tube directly to a draw-bench and there passing it

40 through a die and over a mandrel disposed interiorly of said die and tube, applying a liquid non-water-bearing lubricant simultaneously to both the interior and the exterior surfaces of 45 said tube as it is being drawn through said die and prior to their passage therethrough, and alternately annealing and redrawing said tube without intermediate pickling until the desired diameter and wall thickness are obtained.

55

ELMER N. SANDERS.